

Aug. 26, 1947.

R. H. NEWTON

**2,426,233**

## PRODUCTION OF AVIATION BASE FUEL

Filed March 28, 1942



## UNITED STATES PATENT OFFICE

2,426,233

## PRODUCTION OF AVIATION BASE FUEL

Roger H. Newton, Bowling Green, Pa., assignor  
to Houdry Process Corporation, Wilmington,  
Del., a corporation of Delaware

Application March 28, 1942, Serial No. 436,547

6 Claims. (Cl. 196—52)

1

This invention relates to the production of desirable hydrocarbon materials, including motor fuels and especially base material for high quality, high octane aviation gasoline of the fighting grade type. In certain respects it may be considered as an improvement upon or further development of the invention disclosed in my copending application Serial No. 427,409, filed January 20, 1942.

One object of the invention is to produce high quality hydrocarbon materials having definite characteristics. Another object is to produce aviation base material which can be brought to an octane rating of 100 or better by the addition of tetraethyl lead alone. Other objects will be apparent from the detailed description which follows.

In order to illustrate the invention one concrete embodiment thereof is indicated diagrammatically in the single figure of the accompanying drawing.

In the drawing fresh charge such as gas oil is sent by line 1, along with recycle material added by line 2 through vaporizing still 3, whence it passes at cracking temperature to a catalytic converter 4 containing high activity cracking catalyst. The cracked products pass by line 5 to suitable fractionating equipment such as tower 6 which divides the same in to: (1) a bottoms fraction, which is a clean stock higher boiling than motor gasoline, suitable for use as Diesel oil or domestic fuel oil, which leaves the tower by line 7 to storage in tank 8; (2) a side stream fraction having an end point in the range of 325 to 475° F. which leaves tower 6 by line 9 to pass to a side stream stripper, preferably of the reboiler type which feeds back into tower 6 at a higher level by line 11; and (3) an overhead cut having an end point in the range of 180 to 260° F. which leaves tower 6 by line 12. The side stream fraction leaves stripper 10 by line 13 which is branched to send a portion back to still 3 by line 2 as recycle while the remainder is added to the overhead cut in line 12 and passes with the same either to condenser 14 and gas separator 14a, which are optional and utilized only when lighter products of the first stage of the operation are to be withdrawn, or by by-passing line 15 to further treatment in the second stage of the operation.

2

The condensed hydrocarbons from gas separator 14a or by-pass line 15, or both, which comprise motor gasoline are now subjected to another catalytic treatment in vapor phase under conditions as severe as in the first catalytic cracking zone 4 and usually more severe, as higher temperatures, higher pressures, or both. To this end they are sent through vaporizing still 16 to catalytic converter 17 containing high activity cracking catalyst of the same or different type as in zone 4 and preferably of at least as high activity. The products pass to fractionating equipment such as tower 18 which divides the same according to the desires or requirements of the refiner. In the arrangement shown in the drawing three cuts are made. Aviation base material, 300° F. end point, is taken overhead by line 19 to condenser 20 and thence to separator 21 where fixed gases are removed by line 22 and the aviation gasoline passes by line 23 to suitable stabilizing equipment (not indicated) and thence to storage tank 24. A side stream fraction of motor naphtha, boiling range 300° to 400° F., is removed by line 25 to storage tank 26. The remaining hydrocarbons boiling above 400° F. are removed by bottom line 27 and pass to storage tank 28. The latter are highly aromatic, are highly desirable as solvent, and have other uses of a specialized character.

Any known or suitable forms of catalytic equipment which give proper control of operating conditions may be utilized at 4 and 17. With stationary catalyst, which is preferred, there will be a battery of converters at each location to permit regeneration of the catalytic material in place and to provide for continuous operation. Known catalysts which are highly selective and highly active in promoting cracking reactions are utilized for both zones. Silicious catalysts including silica-alumina blends or compounds, are suitable, preferably those of high purity and synthetically produced, with or without the inclusion of other active materials such as metals or metallic compounds. Zirconium compounds with silica and with or without alumina are also effective catalysts. They should have an activity index of at least 35, which indicates ability to convert at least 35% of a standard reference stock, such as East Texas gas oil under standard operating conditions to lighter products in ac-

cordance with the procedure set forth in detail on page 2 of the specification of United States Patent No. 2,347,216, issued April 25, 1944, to Albert G. Peterkin.

The operating conditions in the first catalytic zone comprise cracking temperature above 750° F. with low or moderate pressures, but subatmospheric pressures may also be used. The combined charge to still 3, fresh and recycle, ranges from 1/2:1 to 3.5:1 (liquid volume of charge per hour per volume of catalyst) and the ratio of recycle to fresh charge may vary from 1/4:1 to 1:1 but is preferably 1/2:1 to 3/4:1. While with certain charging stocks it is possible in the first stage of the operation to take practically a full aviation gasoline overhead in the first fractionating zone and to recycle a side stream cut from the two top trays of the tower, which side stream will overlap somewhat with the overhead cut, it is usually desirable that the recycled material have an initial boiling point of about 200° to 240° F. and an end boiling point of about 400 to 425° F.

As previously stated the operating conditions in the second catalytic zone are usually somewhat more severe than in the first catalytic zone. The temperature will be above 775° F. and usually above 800° F. with superatmospheric pressures of at least 50 lbs. per square inch gauge and usually 75 lbs. or above. The feed rate (liquid volume of charge per hour per volume of catalyst) is not over 1 1/4:1 and is frequently as low as 1/2:1 but is usually from 3/4:1 to 1:1.

Details of a typical operation are given below:

*Example*

The fresh feed to the operation was an East Texas gas oil of 36° A. P. I. gravity and the following boiling range:

|         | °F. |
|---------|-----|
| Initial | 432 |
| 10%     | 480 |
| 50%     | 538 |
| 90%     | 640 |

It was subjected to the action of a synthetic silica-alumina catalyst of high activity (40 index) maintained at a mean temperature of 820° F. under 30 lbs. per square inch gauge pressure for on-stream periods of ten minutes. The total feed rate to the catalyst was 21:20 (liquid volume of charge per hour per volume of catalyst) which was made up of fresh feed 14:20 and recycle stock 7:20, or at a recycle ratio of 1/2:1. The recycle material was a naphtha of the following boiling range:

|         | °F. |
|---------|-----|
| Initial | 230 |
| 10%     | 267 |
| 50%     | 318 |
| 90%     | 402 |

The material charged to the second catalytic zone was approximately 42% of the fresh charge to the first catalytic zone and had the following boiling range:

|         | °F. |
|---------|-----|
| Initial | 82  |
| 10%     | 103 |
| 50%     | 185 |
| 90%     | 360 |

The second catalytic zone containing synthetic silica-alumina catalyst of the same type and ac-

tivity as the first zone and the operating conditions were; mean catalyst temperature 830° F., pressure 75 lbs. per square inch gauge with 1:1 feed rate for on-stream periods of twenty minutes. The yields of both zones were taken for purposes of comparison and were as follows:

|    | Yields in Per cent of Charge to Zone             | First Catalytic Zone | Second Catalytic Zone |
|----|--------------------------------------------------|----------------------|-----------------------|
| 10 |                                                  |                      |                       |
|    | Gas, per cent Weight.....                        | 18.7                 | 11.2                  |
|    | Coke, grams per liter of catalyst.....           | 6.5                  | 3.9                   |
|    | Coke, per cent by weight of charge oil.....      | 6.6                  | 1.5                   |
|    | Liquid recovery.....                             | 79.5                 | 87.1                  |
| 15 | Aviation gasoline debutanized 275° F. @ 90%..... | 35.7                 | 70.6                  |
|    | Motor Naphtha.....                               | 5.8                  | 14.5                  |
|    | Fuel Oil (440-650° F. boiling range).....        | 38.0                 | 12.0                  |

<sup>1</sup> Solvent.

Inspection and tests of the aviation cut of gasoline from each zone revealed the following:

|    | 90% Evaporation at.....                                         | 275° F. | 262° F.                                 |
|----|-----------------------------------------------------------------|---------|-----------------------------------------|
|    | Reid Vapor Pressure.....                                        | 8.3     | 7.6                                     |
|    | Acid Heat.....                                                  | 21      | Less than 5.                            |
| 25 | A. F. D.-I-C Octane +3 cc. T. E. L.....                         | 95.6    | Over 100 or iso-octane+.05 cc. T. E. L. |
|    | +4 cc. T. E. L.....                                             | 97.6    | Over 100 or iso-octane+.02 cc. T. E. L. |
|    | Calculated A. F. D.-I-C Octane at 7 R. V. P.+4 cc. T. E. L..... | 96.8    | Over 100 or iso-octane+.02 cc. T. E. L. |

30 In order to reach 100 octane with the aviation gasoline from the first catalytic stage it was found necessary to add 20% alkylate in addition to the 4 cc. T. E. L.

35 With gas oil charging stock of naphthenic Coastal types the aviation octanes obtainable in each stage will be somewhat higher than in the above example. Mid-Continent gas oils have been found to give approximately the same results as East Texas stocks.

40 It is preferable from an economical standpoint to send the entire motor gasoline cut from the first catalytic stage to the second catalytic stage because of the increased yield of aviation gasoline but it is to be understood that if the aviation cut alone is charged to the second catalytic stage the resulting products will be of like quality. It is particularly to be noted that with 4 cc. of tetraethyl lead the aviation base material from the second stage becomes a finished aviation gasoline having an octane rating considerably above 100, the measure of which is expressed accurately, as indicated in the above example, as iso-octane + tetraethyl lead (fractional cc.'s of tetraethyl lead mean several octane points due to the high lead susceptibility of iso-octane).

I claim as my invention:

1. In the production of high grade fuels of the gasoline type including aviation fuels, the process comprising subjecting hydrocarbon charging stock to catalytic cracking in the presence of a body of highly active cracking catalyst, separating from products of said cracking a light normally liquid distillate having an end point in the range of 180° F. to 260° F. and a heavier distillate having a boiling range from approximately the end point of said light distillate to a temperature within the range of 325° F. to 475° F., returning a portion only of said heavier distillate to said first body of catalyst with said hydrocarbon charging stock, subjecting said light distillate and the remainder of said heavier distillate to catalytic cracking in the presence of a second body of highly active cracking catalyst, and separating a product of the gasoline type

from the products of the last named cracking step.

2. In the catalytic conversion of hydrocarbons, the steps comprising subjecting hydrocarbon charge heavier than gasoline to catalytic cracking in the presence of a body of high activity cracking catalyst, separating from resulting cracked products a first liquid distillate fraction having an end point in the range of 180° F. to 260° F. and a heavier liquid distillate fraction having a boiling range from approximately the end point of said first distillate fraction to a temperature within the range of 325° F. to 475° F., returning a portion only of said heavier liquid distillate to said body of catalyst with said charge for conversion with the latter, combining said first distillate with the balance of said heavier distillate, subjecting the combined distillates to further catalytic cracking in a second separate catalytic cracking step at cracking conditions more severe than used in the first mentioned catalytic cracking step, and separating from products of said second separate catalytic cracking step a high octane distillate of the gasoline type.

3. In the production of high grade fuels of the gasoline type including aviation fuels, the process comprising subjecting hydrocarbon charging stock to catalytic cracking in the presence of high activity cracking catalyst, separating from products of said cracking a relatively heavy gasoline type fraction comprising part only of the cracked hydrocarbons boiling above about 180° F. and below about 475° F., returning said fraction to said cracking catalyst with said hydrocarbon charging stock, subjecting to a second separate catalytic cracking step cracked gasoline type distillate obtained from said first catalytic cracking step, including relatively light gasoline hydrocarbons boiling below about 180° F. and relatively heavy gasoline hydrocarbons boiling within the range of an initial boiling point of approximately 180° F. to 260° F. and an end boiling point of approximately 325° F. to 475° F., and separating from the products of said second catalytic cracking step a high anti-knock liquid product of the gasoline type.

4. In the production of high grade fuels of the gasoline type including aviation fuels, the process comprising subjecting hydrocarbon charging stock to catalytic cracking in the presence of high activity cracking catalyst, separating from products of said cracking a relatively heavy gasoline type fraction comprising part only of the cracked hydrocarbons boiling above about 180° F. and below about 475° F., returning said fraction to said cracking catalyst with said hydrocarbon charging stock in the ratio of one-fourth to one part of said fraction to each part of said hydrocarbon charging stock, subjecting to a second separate catalytic cracking step cracked gasoline type distillate obtained from said first catalytic cracking step, including relatively light gasoline hydrocarbons boiling below about 180° F. and relatively heavy gasoline hydrocarbons boiling within the range of an initial boiling point of approximately 180° F. to 260° F. and an end boiling point of approximately 325° F. to 475° F., and separating from the products of said second catalytic cracking step a high anti-knock liquid of the gasoline type.

5. In the production of high grade fuels of the gasoline type including aviation fuels, the process comprising subjecting hydrocarbon charging

stock to catalytic cracking in the presence of high activity cracking catalyst, separating from products of said cracking a relatively heavy gasoline type fraction comprising part only of the cracked hydrocarbons boiling above about 180° F. and below about 475° F., returning said fraction to said cracking catalyst with said hydrocarbon charging stock, subjecting to a second separate catalytic cracking step effected at cracking conditions more severe than employed with said hydrocarbon charge cracked gasoline type distillate obtained from said first catalytic cracking step, including relatively light gasoline hydrocarbons boiling below about 180° F. and relatively heavy gasoline hydrocarbons boiling within the range of an initial boiling point of approximately 180° F. to 260° F. and an end boiling point of approximately 325° F. to 475° F., and separating from the products of said second catalytic cracking step a high anti-knock liquid product of the gasoline type.

6. In the production of high grade fuels of the gasoline type including aviation fuels, the process comprising subjecting hydrocarbon charging stock to catalytic cracking in the presence of high activity cracking catalyst, separating from products of said cracking a relatively heavy gasoline type fraction comprising part only of the cracked hydrocarbons boiling above about 180° F. and below about 475° F., returning said fraction to said cracking catalyst with said hydrocarbon charging stock, subjecting to a second separate catalytic cracking step effected at higher temperatures and lower space rate than employed with said charging stock cracked gasoline type distillate obtained from said first catalytic cracking step, including relatively light gasoline hydrocarbons boiling below about 180° F. and relatively heavy gasoline hydrocarbons boiling within the range of an initial boiling point of approximately 180° F. to 260° F. and an end boiling point of approximately 325° F. to 475° F., and separating from the products of said second catalytic cracking step a high anti-knock liquid product of the gasoline type.

ROGER H. NEWTON.

#### REFERENCES CITED

50 The following references are of record in the file of this patent:

#### UNITED STATES PATENTS

| Number       | Name                                 | Date                              |
|--------------|--------------------------------------|-----------------------------------|
| 55 2,224,840 | Story -----                          | Dec. 10, 1940                     |
|              | Egloff -----                         | May 12, 1942                      |
|              | Penisten -----                       | Aug. 25, 1942                     |
|              | Houdry -----                         | Dec. 27, 1938                     |
|              | D'Ouville -----                      | Dec. 16, 1941                     |
| 60 2,276,081 | McGrew -----                         | Mar. 10, 1942                     |
|              | 2,283,854                            | Friedman et al. May 19, 1942      |
|              | 2,287,940                            | McGrew ----- June 30, 1942        |
|              | 2,304,183                            | Layng et al. ----- Dec. 8, 1942   |
|              | 2,328,754                            | Thomas ----- Sept. 7, 1943        |
| 65 2,310,327 | Sweeney -----                        | Feb. 9, 1943                      |
|              | 2,337,640                            | Burgin ----- Dec. 28, 1939        |
|              | 2,339,918                            | Thomas ----- Jan. 25, 1944        |
|              | 2,349,045                            | Layng et al. ----- May 16, 1944   |
|              | 2,361,138                            | Voorhies, Jr. ----- Oct. 24, 1944 |
| 70 2,361,611 | D'Ouville et al. ----- Oct. 31, 1944 |                                   |

#### FOREIGN PATENTS

| Number  | Country      | Date         |
|---------|--------------|--------------|
| 829,582 | French ----- | Apr. 5, 1938 |